

June 6, 1967

P. GALLAGHER

3,323,961

METHOD AND APPARATUS FOR FORMING ROD-SHAPED FIBROUS ELEMENTS

Filed Oct. 10, 1963

2 Sheets-Sheet 1



FIG. 1.



FIG. 2.

PAUL GALLAGHER  
INVENTOR

BY *R. Frank Smith*  
*Alvan W. Fletcher*  
ATTORNEYS

June 6, 1967

P. GALLAGHER

3,323,961

METHOD AND APPARATUS FOR FORMING ROD-SHAPED FIBROUS ELEMENTS

Filed Oct. 10, 1963

2 Sheets-Sheet 2



FIG. 4.



FIG. 3.



FIG. 5.

PAUL GALLAGHER  
INVENTOR

BY *R. Frank Smith*  
*Adam W. Hatchett*  
ATTORNEYS

## 1

3,323,961

**METHOD AND APPARATUS FOR FORMING ROD-SHAPED FIBROUS ELEMENTS**

Paul Gallagher, Kingsport, Tenn., assignor to Eastman Kodak Company, Rochester, N.Y., a corporation of New Jersey

Filed Oct. 10, 1963, Ser. No. 315,282  
3 Claims. (Cl. 156—180)

This invention involves a method and apparatus for improving the uniformity of rod-shaped fibrous elements such as tobacco smoke filters. In particular, it involves a method and apparatus for controlling the uniformity of continuous filament tow introduced to a garniture or other rod-forming means.

In U.S. Patent No. 3,016,945 my co-worker Wexler disclosed a method and apparatus for conducting spread-out crimped filaments through a cone-shaped air jet into an immediately adjacent filter element forming means. In U.S. Patent No. 3,050,430 I disclosed an apparatus and process for an improvement over the Wexler method and apparatus for compacting and forming filaments into filter elements wherein the motivating jet employs a venturi portion in immediately adjacent association with a perforated tongue section of the forming means. Although both of these jet arrangements for introducing filter tow into compacting means have proved highly successful in the filter products industry, it has been found desirable in some instances to occasionally interrupt the filter-forming operation to adjust the apparatus to help control uniformity of the circumference of the rod-shaped elements. Accordingly, development of a process and apparatus for improving the uniformity, especially with respect to circumference, of filter elements or other rod-like objects produced by compacting a bundle of continuous filament tow by garniture or other shaping means, represents a highly desirable result. After extended investigation we have found a method and apparatus for improving the uniformity of filter elements and the like not only with respect to circumference of the filter elements but also with respect to pressure drop and weight.

One object of the present invention is to provide a method and apparatus for increasing the uniformity of rod-shaped fibrous elements made from continuous filament tow. Another object is to provide a method and apparatus for improving the uniformity of continuous filament tow as it is introduced from feed rolls to garniture or other compacting means. A further object is to provide a method and apparatus for improving the weight, circumference and pressure drop uniformity of rod-like elements produced by compacting continuous filament tow. Further objects will appear hereinafter.

In the broader aspects of my invention I have found that if prior to the pushing or pulling a bundle of opened-up crimped continuous filaments into compacting and forming means, the bundle of filaments is first conducted through an orifice or constriction associated with means for motivating the bundle of filaments, an improvement in the uniformity, particularly with respect to circumference, of the resulting rod-shaped elements may be obtained. According to my invention the exact size or shape of the orifice or constriction is not controlling, provided it is used in association with means for motivating the continuous filament tow therethrough. Such

## 2

motivating means may include an endless belt, one or more pairs of driven rolls or a similar device. The orifice may be formed simply by two opposing blocks or it may be in the nature of an eyelet or small hole in a narrow barrier. When the orifice consists of a channel rather than a single opening the channel may have parallel sides or may be tapered. In a preferred embodiment the motivating means comprise a jet such as the abovementioned jet of Gallagher U.S. Patent 3,050,430. However, according to the instant invention the jet serves both as orifice and motivating means, the motivating means being fluid introduced into the jet. Rather than being in immediately adjacent juxtaposition with the forming means as in Gallagher U.S. Patent 3,050,430, according to the present invention the jet is positioned between one or more pairs of feed rolls and the relatively remote compacting means.

In a further embodiment of my invention a flattened horn-like structure may be used for introducing the tow uniformly to the compacting means instead of a cone-shaped structure such as that of Wexler U.S. 3,016,945 or Gallagher U.S. 3,050,430.

For a further understanding of my invention reference is made to the attached drawing forming a part of the present application.

FIG. 1 is a semidiagrammatic side elevation view of apparatus for filter element manufacture comprising a filter-forming device having in combination therewith tow constricting means.

FIG. 2 is also a semidiagrammatic side elevation view somewhat on an enlarged scale for clarity showing the constriction means in section.

FIGS. 3 and 4 are schematic representations of an alternate embodiment of the constriction means and associated motivating means of this invention.

FIG. 5 is a perspective view of the forming member or compacting device which may be used for compacting the tow according to the present invention after passage through the constricting means.

FIG. 1 will now be described in detail. In this description the figure will be considered from right to left. Namely, it will be assumed that a bundle of crimped continuous filaments has been obtained and is being fed through the apparatus of FIG. 1 for forming a filter element. In other words, the description will be of a path through the apparatus for forming the spread-out continuous filaments into a compacted filter element.

Therefore, 10 designates the crimped continuous filament tow in a spread-out condition to be made into a filter element. This band of filaments will comprise several thousand individual continuous crimped filaments which have previously been treated in certain desired manner. That is, these filaments may be fluffed, opened up by rolls, sprayed with plasticizer and the like. Further details concerning such treatment may be had from a review of the U.S. Patent 2,794,480 to my coworkers Crawford and Stevens. These filaments 10 pass over and around rolls 12 and 14 for motivating the filaments from the previous treatments such as fluffing, plasticizing, etc. to the treatment by the present invention. These several thousand filaments then arrive at a position designated 16 prior to being passed through the constriction 18 according to the present invention. Since various constructions of this constriction 18 are covered in detail in connection with FIGS. 2, 3 and 4, further detail with respect

to the structure thereof will not be given at this point. After passage through constriction 18 of continuous filaments is moved through the relatively remote compacting device 20 and into a forming and wrapping section generally indicated as 21 including tongue member 22. This compacting device or forming member 20 may be shaped as depicted in FIG. 5. The bottom portion of tongue member 22 may be opened to some extent or otherwise constructed to accommodate an endless belt 24. This belt is driven by drum 26. The belt passes over and under various rollers 28, 30, 32 and 34 whereby the belt rotates under forming member 20 as a conveyor for conveying the formed filter rods through the process. The aforementioned driving drum and rollers are suitably positioned as shown in the drawing so that the belt passes under forming member 20 in a reasonably parallel manner.

Also positioned in association with forming and wrapping section 21 and above belt 24 is a web of wrapping material 36 such as paper. This wrapping material is fed from supply roll 38 under and over suitable guide rolls 40 and 42. As shown in the drawing the wrapping material is brought into continuous contact with the formed filter element in a manner that the filter element may be enclosed in the wrapping material.

At the other end of the apparatus, parts of which have just been described, there is positioned a paste wheel 44, guide bars 46, sealing means 48 and a cutting device 50. These various parts in the order mentioned serve to apply adhesive to the edges of the wrapping material, to fold over the wrapping material, to seal the wrapped filter element and then cut it into suitable lengths. Since these particular parts and their function may be generally in accordance with the corresponding parts shown in above-mentioned Patent No. 2,794,480, extended description herein appears to be unnecessary.

Attention is now turned to FIG. 2, wherein a preferred embodiment of the constriction and motivating device of the present invention is shown. In this embodiment the constriction and motivating means are substantially the same as in the jet depicted in Gallagher U.S. 3,050,430 with the exception that the jet in this instance is positioned as indicated in FIG. 1, that is, between the feed rolls and compacting means rather than in immediately adjacent association with the compacting or filter forming means. An alternate construction of this jet embodiment of constriction and motivating means according to my invention is shown in Wexler U.S. Patent No. 3,016,945 referred to above.

Constriction jet 52 preferably is of cone-shaped construction. That is, the jet overall can be considered somewhat as a truncated cone shape thereby having a considerably greater cross-section on the entrance end 54 than on

the exit end 56. The jet is made up of the inner member 58 and the outer member 60. These parts are suitably threaded at 62 or otherwise fabricated so that they may be assembled together and provide the chamber 64 which encircles the entire inner member. An opening into this chamber is provided at 66 for the introduction of air or other motivating fluid. The inner walls of this chamber are shaped so as to provide an outlet orifice 68 around the periphery of the inner member. In other words, this outlet orifice permits the air or the like motivating gas to escape out through the exit end 56 of the jet. The size of this outlet orifice may be determined by the thickness of gasket 70.

In FIG. 3 orifice 72 comprises two block-like portions 15 74 and 76 positioned opposite each other providing a constricted channel 78 for passage of tow 80 therethrough. A tapered section 82 is provided for introducing tow to orifice 72 through a funnel-shaped channel 84. Immediately downstream from said orifice 72 are located two 20 endless belts 86 and 88 position so as to move the band of tow 90 therebetween after it leaves orifice 92 and to conduct it therefrom toward forming means such as 20 shown in FIG. 1.

Referring now to FIG. 4, in an alternate embodiment 25 a band of tow 94 is introduced through orifice 96 having a tapered portion 98 which gradually decreases in size to the smallest point 100 and a uniform size portion 102. After passing through channels 98 and 102 of orifice 96 the tow is motivated therefrom toward compacting means 20 such as that of FIG. 1 by moving between the nip of rolls 104 and 106.

A still further understanding of my invention will be had from a consideration of the following examples which are set forth for illustrating certain preferred embodiments 30 of the instant invention.

#### EXAMPLE I

A series of samples (approximately 50 of each type) 40 of tow was conducted through an orifice jet such as that illustrated in FIG. 2 and then compacted into tobacco smoke filters. Measurements were made and averages recorded as indicated in the following table of the rod weight, circumference, circumference standard deviation, 45 plasticized tow weight, weight standard deviation, pressure drop and pressure drop standard deviation. The table also reports similar data for a sample conducted through the compacting device without first being passed through an orifice such as that of the present invention. The improvement in uniformity of the filters by the process and apparatus of this invention is demonstrated by the data 50 in this table.

TABLE I

| Sample      | Tow Weight, 1 Rod (g.) | Circ. (mm.)        | St'd.Dev. in Circ. | Circ. (mm)        | St'd. Dev. Circ. | Plasticized Tow Weight (g.) | St'd. Dev. Press. Drop (in H <sub>2</sub> O) <sup>4</sup> | St'd. Dev. in Press. | Rod Size (mm.) | Diameter of Orifice, inch | Tow              |                  |
|-------------|------------------------|--------------------|--------------------|-------------------|------------------|-----------------------------|-----------------------------------------------------------|----------------------|----------------|---------------------------|------------------|------------------|
| Control A-1 | .763                   | <sup>1</sup> 24.7  | .083               | <sup>3</sup> 24.8 | .103             | .836                        | .0116                                                     | .551                 | 24.7 x 102     | <sup>3/8</sup>            | 3D/F, 57,000 TD. |                  |
|             | .768                   | <sup>1</sup> 24.7  | .063               | <sup>3</sup> 24.9 | .056             | .842                        | .0089                                                     | .11.9                | .418           | <sup>3/8</sup>            | 3D/F, 57,000 TD. |                  |
| Control B-  | .856                   | <sup>2</sup> 24.78 | .090               | -----             | -----            | -----                       | .0284                                                     | 10.6                 | .588           | -----                     | 5D/F, 60,000 TD. |                  |
|             | .856                   | <sup>2</sup> 24.81 | .085               | -----             | -----            | -----                       | .0276                                                     | 10.8                 | .322           | 24.8 x 102                | <sup>1/2</sup>   | 5D/F, 60,000 TD. |
|             | .853                   | <sup>2</sup> 24.79 | .061               | -----             | -----            | -----                       | .0256                                                     | 11.1                 | .273           | 24.8 x 102                | <sup>1/2</sup>   | 5D/F, 60,000 TD. |

## NOTES:

<sup>1</sup> By measuring seam width microscopically.

<sup>2</sup> By standard air gage method.

<sup>3</sup> By measuring with print method.

<sup>4</sup> By measuring resistance to flow of 17.5 ml. air per second through rod.

Circ. = Circumference.

St'd. = Standard.

Dev. = Deviation.

Press. = Pressure.

**5**  
**EXAMPLE II**

A series of samples of tow was formed into filter elements by passing through a fish-mouthed or flattened cone horn guide such as that depicted in FIG. 5 and physical properties measured similar to those in Table I. The results are shown in the following table. These results were compared with those for controls passed through a conical-shaped horn or forming device as also reported in the following table.

5

6

comprises a constriction orifice and motivating means positioned between said roll means and said compacting and forming means whereby the filaments are shaped into a band of uniform width, said orifice being positioned relatively closer to said roll means than to said compacting and forming means.

2. An apparatus in accordance with claim 1 wherein the constricting orifice in association with motivating means comprises a jet having a large open end positioned

TABLE II

| Sample    | Denier (DF/TD) | Size (mm.) | Tow Wt., 1 Rod (g.) | Pressure Drop (mm.) | Standard Deviation Press. Drop (mm.) | Avg. Circ. (mm.) | St'd. Dev. Circ. | Type of Apparatus                                   |
|-----------|----------------|------------|---------------------|---------------------|--------------------------------------|------------------|------------------|-----------------------------------------------------|
| Control A | 3/53           | 24.8 x 78  | .574                | 9.7                 | .266                                 | 24.86            | .051             | 2 piece tongue+standard horn.                       |
| Control B | 3/53           | 24.8 x 78  | .574                | 9.7                 | .303                                 | 24.87            | .061             | 1 piece tongue+standard horn.                       |
| 1         | 3/53           | 24.8 x 78  | .573                | 9.9                 | .362                                 | 24.86            | .078             | 1 piece tongue+1/8" fishmouth horn.                 |
| 2         | 3/53           | 24.8 x 78  | .573                | 9.8                 | .229                                 | 24.88            | .058             | 1 piece tongue+5/8" fishmouth horn.                 |
| Control C | 3.3/46         | 24.8 x 102 | .743                | 17.3                | .517                                 | 24.83            | .059             | 2 piece tongue+standard horn.                       |
| Control D | 3.3/46         | 24.8 x 102 | .738                | 16.0                | .861                                 | 24.77            | .070             | 1 piece tongue+standard horn.                       |
| 1         | 3.3/46         | 24.8 x 102 | .661                | 12.4                | .565                                 | 24.76            | .089             | 2 piece tongue+1/2" fishmouth horn (rods wrinkled). |
| 2         | 3.3/46         | 24.8 x 102 | .714                | 15.3                | .654                                 | 24.77            | .044             | 2 piece tongue+1/2" fishmouth horn.                 |
| 3         | 3.3/46         | 24.8 x 102 | .713                | 14.3                | .480                                 | 24.82            | .075             | 1 piece tongue+1/2" fishmouth horn.                 |
| 4         | 3.3/46         | 24.8 x 102 | .662                | 12.6                | .362                                 | 24.85            | .066             | 1 piece tongue+1/2" fishmouth horn (rods wrinkled). |
| Control E | 3.3/46         | 24.8 x 102 | .745                | 15.9                | .928                                 | 24.82            | .050             | 2 piece tongue+standard horn.                       |
| Control F | 5/60           | 24.8 x 102 | .943                | 11.9                | .654                                 | 24.84            | .188             | 2 piece tongue+standard horn.                       |
| 5         | 5/60           | 24.8 x 102 | .889                | 11.0                | .661                                 | 24.87            | .133             | 2 piece tongue+5/8" fishmouth horn.                 |
| 6         | 5/60           | 24.8 x 102 | .838                | 9.0                 | .554                                 | 24.90            | .105             | 2 piece tongue+1/2" fishmouth horn (rods wrinkled). |
| 7         | 5/60           | 24.8 x 102 | .863                | 10.0                | .433                                 | 24.84            | .120             | 1 piece tongue+1/2" fishmouth horn (rods wrinkled). |
| 8         | 5/60           | 24.8 x 102 | .899                | 10.5                | .654                                 | 24.79            | .111             | 1 piece tongue+1/2" fishmouth horn.                 |
| Control G | 5/60           | 24.8 x 102 | .905                | 12.0                | .909                                 | 24.88            | .100             | 1 piece tongue+standard horn.                       |
| Control H | 5/60           | 24.8 x 102 | .856                | 10.6                | .588                                 | 24.78            | .090             | 2 piece tongue+st'd. horn+st'd. 6 day glue.         |
| 9         | 5/60           | 24.8 x 102 | .856                | 10.8                | .322                                 | 24.81            | .085             | 2 piece tongue+st'd. horn+5/8" stuffer 6 day glue.  |
| 10        | 5/60           | 24.8 x 102 | .853                | 11.1                | .273                                 | 24.79            | .061             | 2 piece tongue+st'd. horn+5/8" stuffer 6 day glue.  |

From the foregoing description and examples it is thought apparent that I have provided by my invention a method and apparatus for improving the uniformity of weight circumference, and pressure drop of filter elements prepared by passing a band of spread-out continuous filament tow through forming means, said improvement being accomplished by passing the tow through a confining means such as an orifice or constriction and either as a part thereof or in association therewith, motivating means.

The invention has been described in detail with particular reference to preferred embodiments thereof, but it will be understood that variations and modifications can be effected within the spirit and scope of the invention as described hereinabove and as defined in the appended claims.

I claim:

1. In an apparatus for manufacture of tobacco smoke filter elements from crimped continuous filaments which comprises roll means for feeding spread-out filaments to compacting and forming means, the improvement which

35

40

45

50

toward the roll means and a small end positioned toward the compacting and forming means, said small end being provided internally with means for the injection of a motivating fluid within the jet whereby the filaments are motivated from the jet to the separate compacting and forming means.

3. An apparatus in accordance with claim 1 wherein the compacting and forming means comprise a tongue-like element having a fishmouth-shaped horn in juxtaposition therewith for introducing the constricted filaments thereto.

**References Cited**

**UNITED STATES PATENTS**

|           |        |               |       |           |
|-----------|--------|---------------|-------|-----------|
| 3,050,430 | 8/1962 | Gallagher     | ----- | 156—166   |
| 3,120,690 | 2/1964 | Stevens       | ----- | 156—166 X |
| 3,144,025 | 8/1964 | Erlich        | ----- | 156—180 X |
| 3,148,101 | 9/1964 | Allman et al. | ----- | 156—180 X |

EARL M. BERGERT, Primary Examiner.

J. P. MELOCHE, Assistant Examiner.